

# UNITED STATES PATENT OFFICE.

EMILE BRONNERT, OF MÜLHAUSEN, ALSACE-LORRAINE, FRANCE.

## MANUFACTURE OF ARTIFICIAL SILK.

1,393,199.

Specification of Letters Patent. Patented Oct. 11, 1921.

No Drawing.

Application filed September 14, 1920. Serial No. 410,141.

To all whom it may concern:

Be it known that I, EMILE BRONNERT, a citizen of the Republic of France, residing at 1 Quai du Barrage, in Mülhausen, Alsace-Lorraine, France, have invented certain new and useful Improvements in the Manufacture of Artificial Silk, of which the following is a specification.

The present process for the manufacture 10 of viscose threads of any fineness, from all sorts of raw viscose and of varying consistency, is characterized by the fact that the absolute concentration of the precipitant baths is adapted to the consistency of the 15 raw viscose, the acid concentration being increased according to the fineness of thread desired and the diameter of the nozzle opening selected to correspond.

In the applicant's former patents it has 20 been shown how success has been obtained in a practical manner in also obtaining the finest threads, of 1 denier for instance, from viscose by means of the apparatus usually employed for ordinary thicker threads of 25 say 8 deniers, by which the threads do not fall to the bottom in the weak precipitant bath, but are drawn upward through a strong precipitant medium.

As is well known according to these 30 proposals in general the concentration of the acid serving for decomposition had to be increased all the more the finer the threads that it was desired to produce.

Less essential in this connection was the 35 quantity, used at the time, of the usual additions to the acids or to the viscose itself if compatible with it, in order to tone down their all-too vigorous action and in order to be able to leave the state of ripeness of the 40 viscose out of consideration to a far reaching extent.

Now for reasons of convenience the technical viscose silk industry has, hitherto, as is well known substantially worked up 45 grades of viscose which contained about 8% cellulose and about 7% caustic soda, although for special purposes not only other proportions between the said ingredients but also higher cellulose concentrations are 50 in any case customary.

In order to obtain the silk threads, hitherto solely produced upon a manufacturing scale in the technical world, of 6 deniers upward to about 10 deniers for each single 55 thread, use was made of the nozzle apertures customary in connection with nitro-

cellulose and ammoniac copper silk of about 0.10 to 0.20 mm, diameter the viscose employed for the purpose, in order to avoid higher pressure being mostly such as can be obtained in any consistency desired for instance by using previously prepared cellulose or by suitable time and temperature measurement or by alteration of the stoichiometric proportions in the manufacture and 65 graduation of the lowering of the molecular weight of the cellulose.

The more consistent the viscose to be worked up is selected, all the wider is it customary to select the nozzle apertures with a 70 view to avoiding unnecessary high pressure.

Now it has been found that with viscose of different consistencies with varying thread titrations or "counts" the concentration of the acid must undoubtedly be relatively adapted to the known regulation conditions but, must however, be taken absolutely all the higher the greater the cross section which has been selected for the nozzle apertures in correlation to the greater 75 consistency of the corresponding viscose. The 80 recognition of this fact is of the greatest importance for the technical man.

### Example 1.

85

A viscose of the usual composition is spun, in the production of which however, the alkali cellulose has experienced in the known manner, a preliminary ripening of 3 days for instance at about 25° C. and which has 90 been sulfidized at the ordinary temperature. After leaving the dissolving-apparatus the viscose is subjected to a further several days subsequent ripening also at an ordinary temperature. It is then somewhat in the nature 95 of a thin liquid (about 100 viscosity units i. e. 100 seconds have been required to allow 100 ccm. of the corresponding viscose to flow out of the cylindrical part of a pipe about 30 mm. wide which is rounded off at the bottom and runs out into a pipe union about 10 mm. long and 3 mm. wide).

For the precipitant bath warm diluted sulfuric acid is used in the known manner to which, essentially for increasing the sheen 105 and softness, there are added one or more of the substances known for this purpose (glucose, sulfates, oxy-acid, poly-atomic alcohols, etc.). The same admixtures can be made to the viscose itself.

The minimum acid concentration of the spinning bath then measured approximately 110

at a fully sufficient spinning length of 10-30 cm.

| 5  | Diameter of apertures mm. | With 7 de-niers gr. H <sub>2</sub> SO <sub>4</sub> pr. liter. | With 4 de-niers gr. H <sub>2</sub> SO <sub>4</sub> pr. liter. | With 2 de-niers gr. H <sub>2</sub> SO <sub>4</sub> pr. liter. |
|----|---------------------------|---------------------------------------------------------------|---------------------------------------------------------------|---------------------------------------------------------------|
| 10 | 0.08                      | 80                                                            | 105                                                           | 150                                                           |
|    | 0.1                       | 125                                                           | 165                                                           | 235                                                           |
|    | 0.13                      | 210                                                           | 280                                                           | 390                                                           |
|    | 0.15                      | 280                                                           | 370                                                           | 520                                                           |

*Example II:*

A viscose is used in the manufacture of which the alkali cellulose divided up into 15 small boxes has been allowed to stand uncovered only a short time after leaving the grinding works or mills in order to acquire a uniform room temperature, the sulfidizing having been carried out up to good solubility under the usual avoidance of increase 20 in temperature and in which the solution was also effected at once without increase of temperature.

As precipitant bath sulfuric acid is again 25 used with the known additions or, in this case, also without such additions. The consistency of a viscose thus prepared is, as is well known, substantially higher and, according to the degree of admissible working, 30 about 1½-3 times higher and even more than in Example 1, so that the spinning of the solution is best effected through nozzle apertures of for example 0.15 mm. and more in diameter. For such more consistent viscose the minimum concentrations of the 35 above tables are preferably considerably exceeded, and, namely, all the more all the higher the consistency of the viscose with an equal percentage of cellulose.

40 The necessary higher acidity is thus shown to be quite convenient, inasmuch as although the decomposing reaction steadily becomes

shorter, it allows the spinning stretch to be maintained as before within the limits of 10 to 30 cm.

45

The use even of relatively highly concentrated acid with such immature and consequently thick viscose is free from objection, as the xanthogenate therein first saponifies but very little and consequently but very 50 little sulfur of sodium is present so that, on decomposing the viscose, no evolution worthy of mention of sulfureted hydrogen takes place, so that it is not necessary to take any steps to render this gas innocuous. The 55 threads arising from the spinning bath are generally covered with a larger quantity of sulfur than in Example I. Moreover after the washings the same can be easily and harmlessly dissolved out.

60

It seems in a highly desirable manner to insure that no all-too-rapid, and consequently under certain conditions, prejudicial, decomposition of the viscose threads takes place.

65

What I claim is:—

The process of producing viscose threads of any desired fineness from raw viscose of various consistencies, which comprises forcing the viscose through suitable openings 70 into an acid precipitating bath, the concentration of which is increased proportionately to the increase in the fineness of the thread desired to be produced, the increase in the consistency of the viscose used, and the increase in the size of the openings through which the viscose is forced.

75

In witness whereof I have hereunto signed my name in the presence of two subscribing witnesses.

EMILE BRONNERT.

Witnesses:

L. R. DE SALIS,  
N. H. MUMBERGER.